

## UNITED STATES PATENT OFFICE

2,341,485

## REDUCING CURL OF PHOTOGRAPHIC FILM

Donald R. Swan, Rochester, N. Y., assignor to  
 Eastman Kodak Company, Rochester, N. Y., a  
 corporation of New Jersey

No Drawing. Application March 28, 1942,  
 Serial No. 436,716

5 Claims. (Cl. 95—88)

This application relates to photography and particularly to a method for reducing the curling tendency of photographic film.

It is well known that photographic film consisting of a cellulosic support carrying one or more emulsion layers has a tendency to curl when used in a photographic projector. Such tendency is especially noticeable in the case of 16 mm. motion picture film in rolls containing 800 feet or more when used, for example, in a repeating projector. Attempts to reduce or overcome this curling tendency of the film by coating layers such as gelatin layers on the reverse side of the film and the incorporation of plasticizers in the gelatin on either side of the film such as glycerol, polyglycerol, nonaethylene glycol and Aquaresin have not been wholly successful. The film exhibits a tendency to curl at high humidity due to the alteration of the water content of the gelatin.

It is, therefore, the object of the present invention to provide a method for overcoming the curling tendency of finished photographic film.

This object is accomplished by the present invention by treating the film after processing, that is, after development and fixing and either before or after drying in an aqueous solution of a water-soluble amide such as urea.

My invention is applicable to the treatment of photographic film consisting of a cellulosic support having thereon a gelatin emulsion layer or layers. The support may be a cellulose ester such as cellulose nitrate, cellulose acetate or cellulose acetate propionate or a cellulose ether or synthetic resin. The emulsion layer in which the image is formed may consist of a gelatin silver halide emulsion or an emulsion using some other water swellable colloidal material such as polyvinyl resin. In addition to the treatment of motion picture film in either 16 millimeter or 35 millimeter widths, my invention is also applicable to the treatment of sheet film or film used in the production of still pictures.

The materials which I propose to use for reducing the curl of finished photographic film are water-soluble amides such as urea, acetamide, formamide, malonamide, lactamide and gluconamide, and mixtures of two or more of these. The film is treated with these materials for a suitable length of time such as by immersion for ten minutes and is then squeegeed and dried.

The preferred water-soluble amide for the treatment of photographic film according to my invention is urea and I prefer to use amounts ranging from 2% to 7.5% in aqueous solution.

If film so treated is to be used at high relative humidities, such as 70-80% relative humidity the amount of urea in the treating bath should not be above 3.5 or 4% by weight. Film soaked in a treating bath above these concentrations is likely to be slightly tacky on the emulsion side at 70-80% relative humidity.

In order to determine the effect of treatment of photographic film according to my invention, I have made the following tests on 16 millimeter motion picture positive film which was flashed and developed and then immersed in solutions of urea of varying concentration. The curling tendency of the film was measured in inches of positive or negative curl, positive curl being used to designate the curling tendency of the edges of the film toward the emulsion side and negative curl to indicate the curling tendency of the edges of the film away from the emulsion side. The "humidity curl amplitude" is the difference between curl at any two relative humidities and may, therefore, be used as a measure of the tendency of the film to curl or conversely to retain its flatness when subjected to variations in humidity.

| Treatment | Curl at   | Curl at   | Humidity       |
|-----------|-----------|-----------|----------------|
|           | 20% R. H. | 70% R. H. | curl amplitude |
| Check     | Inch      | Inch      | Inch           |
| Urea 2%   | +0.065    | -0.005    | 0.060          |
| Urea 2.5% | +0.040    | -0.015    | 0.055          |
| Urea 3%   | +0.060    | -0.005    | 0.055          |
| Urea 4%   | +0.020    | -0.020    | 0.040          |
| Urea 5%   | +0.015    | -0.015    | 0.030          |
| Urea 6%   | +0.005    | -0.025    | 0.030          |
| Urea 7.5% | -0.025    | -0.020    | 0.005          |

These curl measurements were made after two hours' conditioning of the film at the relative humidity indicated and at 70° F. I found that while an increase in the amount of urea in the treating solutions did not always produce a uniform increase in positive or negative curl of the film, the humidity curl amplitude showed a progressive decrease, and a progressive improvement in curling tendency with increasing amounts of urea.

The following example indicates my preferred method of operation: wet or dry processed motion picture film is immersed for ten minutes in an aqueous solution of urea containing 3.5 to 4 parts by weight of the urea to 100 parts by volume of the water. At the end of 10 minutes the film is removed, squeegeed and dried. The operation may, of course, be carried out either as

a discontinuous operation or on a continuous machine.

It will be understood that the examples included herein are illustrative only and that my invention is to be taken as limited only by the scope of the appended claims.

I claim:

1. The method of reducing the curling tendency of finished photographic film which comprises treating said film after processing with an aqueous solution containing from 2% to 7.5% of a water-soluble amide.
2. The method of reducing the curling tendency of finished photographic film which comprises treating said film after processing with a 2% to 7.5% aqueous solution of urea.
3. The method of reducing the tendency of

finished photographic film to curl when subjected to high relative humidity, which comprises immersing said film after development and fixing in a 2% to 7.5% aqueous solution of urea.

5. The method of reducing the tendency of finished photographic film to curl when subjected to high relative humidity, which comprises immersing said film after development and fixing in a 2% to 7.5% aqueous solution of urea.

- 10 5. The method of reducing the tendency of finished photographic film to curl when subjected to high relative humidity, which comprises immersing said film for about 10 minutes 15 in a 2% to 7.5% aqueous solution of urea and then drying said film.

DONALD R. SWAN.